

## UNITED STATES PATENT OFFICE.

HARRY P. BASSETT, OF CYNTHIANA, KENTUCKY, AND THOMAS F. BANIGAN, OF PHILADELPHIA, PENNSYLVANIA, ASSIGNEES TO MEIGS, BASSETT & SLAUGHTER, INC., OF PHILADELPHIA, PENNSYLVANIA, A CORPORATION OF PENNSYLVANIA.

## PROCESS OF FORMING CELLULOSE PRODUCTS.

No Drawing.

Application filed May 11, 1923. Serial No. 638,393.

This invention relates to processes of forming cellulose products, and more particularly to a process of forming finished products from acetyl nitro cellulose in which the acetyl nitro cellulose, while still in the acetylizing solution, is diluted to a desired consistency and then submitted to the usual spinning operation, or other finishing step to produce a desired product.

10 In the use of cellulose acetate or mixtures of cellulose acetate and nitro cellulose, it is customary to remove the material from the acetylizing solution, by precipitation, thus obtaining a solid substantially dry material 15 which is then spun or otherwise treated to produce a finished product.

In a copending application Serial No. 638,391 filed May 11, 1923, we have disclosed and claimed a cellulose material consisting 20 of both nitro and acetyl groups in combination with the cellulose group, a product which is truly an acetyl nitro cellulose. We have found that this material may be spun or otherwise treated to produce a finished 25 product without first removing it from the acetylizing solution by first reducing the consistency of the solution containing the acetyl nitro cellulose to a workable consistency. The fact that this acetyl nitro cellulose may be treated to produce a finished 30 product without first removing it from the acetylizing solution enables us to save considerable time and labor in the production of the finished product.

35 In the preferred practice of the process, the solution obtained when the nitrocellulose is acetylated, consisting of acetyl nitro cellulose in a mixture of acetic acid and acetic anhydride, which is in the form of a 40 thick, viscous jelly obtained from the acetylizing reaction, as described in our copending application, is treated with glacial acetic acid to reduce the consistency to a point where the material may be spun. In place 45 of glacial acetic acid, a weak solution of acetic acid may be employed and a sufficient amount of this weak acetic acid is added to the acetylizing solution, containing the acetyl nitro cellulose to reduce the consistency

to the point where the acetyl nitro cellulose 50 is just about to be precipitated. This material consisting either of the acetylizing solution containing acetyl nitro cellulose which has been treated with acetic acid, or 55 consisting of the acetylizing solution containing acetyl nitro cellulose which has been treated with a weak solution of acetic acid, as above described, may then be spun to produce artificial silk and other filaments or 60 may be treated in the usual manner to form photographic films or other finished products.

In forming artificial silk and other filaments, the material is spun through a precipitating bath. Where the consistency of 65 the solution has been reduced by the use of glacial acetic acid, this bath may consist of a mixture of acetic acid and water, of about 50 to 60 per cent acetic acid. When weak acetic acid has been used to reduce the solution to almost the point of precipitation of the acetyl nitro cellulose, a precipitating bath of very weak acetic acid may be used. In either instance, the spinning mixture can 70 be spun through a precipitating bath of 75 acetic acid and an inert liquid, such as benzol. The benzol, or other inert liquid, is employed to permit recovery of the acetic anhydride contained in the spinning solution. 80

As stated, the fact that this material may be submitted to finishing steps to form finished products without removing it from the acetylizing solution is a material advantage, in that it saves considerable time 85 and labor in the elimination of the precipitating step.

While we have described in detail the preferred practice of our process, it is to be understood that the details of procedure may 90 be widely varied without departing from the spirit of the invention or the scope of the subjoined claims.

We claim:

1. The process of forming cellulose products which comprises bringing an acetylizing solution containing acetyl nitro cellulose 95 to a point just above the precipitating point

of the acetyl nitro cellulose, and then submitting it to a finishing step to produce a desired product.

2. The process of forming cellulose products which comprises bringing an acetylizing solution containing acetyl nitro cellulose to a point just above the precipitating point

of the acetyl nitro cellulose, and then spinning the acetyl nitro cellulose without removing it from the solution.

In testimony whereof, we affix our signatures.

HARRY P. BASSETT.  
THOMAS F. BANIGAN.